

Feb. 27, 1934.

H. A. BRASSET

1,948,697

MANUFACTURE OF METALS

Filed July 27, 1931

2 Sheets-Sheet 1



Feb. 27, 1934.

H. A. BRASSETT

1,948,697

MANUFACTURE OF METALS

Filed July 27, 1931

2 Sheets-Sheet 2



Inventor:  
Herman A. Brassert,  
By: Wilkinson, Shirley, Bryant & Knight  
Atty.

## UNITED STATES PATENT OFFICE

1,948,697

## MANUFACTURE OF METALS

Herman A. Brassert, Chicago, Ill., assignor to  
 H. A. Brassert & Company, Chicago, Ill., a corporation of Illinois

Application July 27, 1931. Serial No. 553,249

2 Claims. (Cl. 75—17)

This invention relates to the manufacture of metals and especially of iron and steel, and more particularly to the production of a purer grade of metal than is usually obtained by the present methods.

It is a well known fact that iron or steel made directly from virgin material, that is from the iron in the ore, without permitting the metal to be reoxidized or to saturate itself with foreign substances, is of a superior quality. In the blast furnace the iron ore is first reduced and then that portion of it which happens to descend in the areas close to the tuyères is reoxidized in the presence of preponderant amounts of oxygen and  $\text{CO}_2$  in the tuyère areas. Such iron oxides are again reduced as they come in contact with the incandescent carbon of the coke lying in the hearth. Whether all of the oxides are reduced depends on the temperature of the hearth, the reactivity of the coke and the time element. At any rate, the effect of the tuyère blast on the reduced iron or molten iron sponge trickling down past the tuyères is detrimental to the quality of the iron, not only in that it is exposed to oxidation but also to the absorption from the blast of hydrogen and nitrogen.

In the blast furnace process, as now carried on, this cannot be prevented as the enormous blast volume required to burn the heavy coke charge penetrates a considerable distance into the coke bed without its oxygen being completely converted into  $\text{CO}$ . The slow reactivity of metallurgical coke aggravates this phenomenon. Charcoal with its high reactivity reduces this oxidizing phase. The gradual increase of hearth diameters has decreased the relative size of the annular oxidizing zone in the tuyère area. However, this increase in hearth diameters has brought with it disadvantages, as for instance a substantial decrease in the productive capacity of blast furnaces per square foot of hearth area, due to the large inert center areas present in such furnaces. Also there are heavy flue dust losses due to the increased volumes of blast required to cover the enormous circumferences of such hearths. The latter objection can be overcome by decreasing the nitrogen content of the blast through oxygen enrichment. This, however, would further aggravate the phase of iron oxidation which is so objectionable and which should be prevented as much as possible.

It is an object of the present invention to provide a new and improved method for the manufacture of a purer grade of metal than is usually obtained by present methods.

It is a further object to provide a method whereby reduction and melting can be carried out in a reducing gas phase throughout.

It is also an object to provide a method for the production of iron or steel whereby the introduction of sulphur into the metal from coke fuel is reduced to a minimum or entirely eliminated.

Other and further objects will appear as the description proceeds.

My invention provides a method whereby reduction and melting can be carried out in a reducing gas phase throughout. This cannot be accomplished if coke is used as a fuel. Coke is too slow to react with the blast, consequently there will always be an oxidizing zone in front of the tuyères when coke is used. The larger the coke and the denser, harder and slower burning it is, the deeper this zone will penetrate toward the center. I propose, therefore, to do away with the method of reducing and melting, as carried out in the present blast furnace, and to substitute a more reactive fuel than coke for carrying out my process. I propose to substantially eliminate the oxidizing zone in the tuyère area.

This I accomplish by substituting for the present blast furnace hearth and bosh a chamber of such dimensions as to provide an annular combustion space around the descending materials. This annular combustion chamber should be of such depth that combustion can be completed to such an extent externally to the mass of materials that no free carbon remains. Into this chamber I feed fuel and combustion air in such proportions that the resulting flame is of a reducing character so that the melting materials will not be re-oxidized in contact with either oxygen or  $\text{CO}_2$ .

I have shown a preferred embodiment of a furnace adapted for carrying out my invention in the accompanying drawings, in which—

Figure 1 is a vertical section through the furnace;

Figure 2 is a horizontal section taken through the lower line of tuyères; and

Figure 3 is a plan view of the hearth portion partly in section, through the upper line of tuyères.

In the drawings, the stack portion 11 is shown as provided with a metal shell 12 and a refractory lining 13, which is provided with water cooled bosh plates 14 which may be of usual construction. It will be understood that any usual type of charging bell may be located at the up-

per end of the stack portion, which will also be provided with offtakes for carrying off the products of combustion.

The stack portion is supported on the annular 5 water cooled metal ring 15. The hearth portion 16 is provided with a base 17 which may be formed of any usual refractory brick or other similar material, and which is enclosed in a water cooled metal jacket 18. The hearth is shown 10 as covered with a lining 19 of refractory material which may be any of the types of material used in open hearth and similar furnaces. A tapping hole 20 is provided for removing the slag and a lower tapping hole 21 provided for use in removing 15 the molten metal.

A plurality of doors 22 are provided at spaced points about the walls adjacent the slag line, these doors serving for cleanout and inspection purposes and also for the addition of any material 20 which it may be desired to add to the bath during the refining process.

The central portion 23 of the hearth is raised and this, together with the layer of refractory material 19 on the central portion, causes this 25 portion to extend to a level above that of the lower line of tuyères 24. These tuyères are fed with air through pipes 25 leading from bustle pipe 26, and with fuel through pipes 27 fed from fuel header 28. As clearly shown in Figure 2, 30 these tuyères 24 are located on approximately tangential lines so that the flame from the tuyères is directed down on the annular bath of metal and slag rather than toward the raised central portion of the hearth. This causes a circular movement of the heated gases and enables 35 the flame to be in contact with the bath over an extended space without burning out the refractory central portion. This refractory central portion 23 may be provided with suitable cooling means, such as the pipes 29, to assist in maintaining it.

The upper curved wall portion 30 of the hearth section is shown as made up of a plurality of segments 31, as best shown in Figure 3. These segments 45 are individually removable, being supported at their upper ends against the water cooled ring 15 and at their lower ends by the water cooled flange 32 of the water cooled jacket 18 of the vertical walls. These segments 31 are provided with a plurality of water cooled pipes 33, and their inner faces are formed by refractory brick 34.

The upper series of tuyères 35 extend through the curved portions, certain segments 36 being 55 especially designed and provided with tuyère openings. The tuyères 35 are fed with air through pipes 37 from the bustle pipe 26, and with fuel through pipe 38 from header 28. As clearly shown in Figure 3, these tuyères 35 are 60 preferably placed slightly off of an exact radial line so as to insure a circulatory movement of the gases and yet they are not placed tangentially as the lower tuyères, as it is desired to direct the flame from the upper tuyères against the central column of descending material.

A third set of tuyères 39 discharge through small openings 40 into the upper portion of the domed section of the hearth. These tuyères 39 are supplied through pipe 41 from the bustle pipe 42. These tuyères are normally supplied with 70 burned gases or other inert gases which will not burn, and which gases form a protective layer adjacent the inner surface of the domed hearth 75 wall to protect this surface against erosion by the

heated products of combustion from the two lower sets of tuyères.

It is well known that the temperatures required for melting pure iron are very much higher than for iron containing carbon. As I propose to 80 limit the amount of carbon absorbed in the melting iron, and as I desire to use a reducing flame, which means incomplete combustion of the fuel, I propose to use much higher air temperatures than are used or necessary in present blast fur- 85 nace practice.

In fact the carrying out of my invention to its fullest extent has become possible through the recent development of means of economically producing high blast temperatures, such means 90 consisting of zoned checkerwork, as described in Patents No. 1,771,282, July 22, 1930, and No. 1,771,286, July 22, 1930. Preferably I heat the air to 1800° F. and as much more as possible before admitting it to the tuyères. The high blast 95 temperatures compensate for the loss of flame temperature caused by carrying a reducing flame. The fuel used for the purpose of obtaining 100 and maintaining a reducing phase in the melting zone is preferably powdered coal, which may be injected by itself or as an addition to other fuels, such as natural gas, coke oven gas, blast furnace gas, producer gas or oil.

As a means for better control of my process, I 105 may also use a blast enriched with oxygen preferably to about twice its natural content. This can be done very economically by modern methods, and has the advantage of considerably increasing the flame temperature. This permits me to carry a flame with a still greater excess of 110 carbon producing a phase of stronger reducing power, which will accelerate the reduction of the ores without retarding the melting process. It will also result in a still finer grade of iron being 115 made, as my iron is protected from the direct action of the enriched blast.

A further important advantage of the use of fuels of this character lies in the fact that the sulphur which is normally introduced into the metal from the usual coke fuel charge, is not 120 brought into the process. This sulphur is injurious to the iron and its removal adds to refining costs so that its elimination at its source is highly desirable.

To follow the process through, when using ore, 125 I charge it into the top of the furnace. It descends through the shaft in contact with the CO ascending from the reducing gas phase below, which gives off its heat to the descending materials and reduces same by indirect reduc- 130 tion. I add some carbon to the ore charge to cause some direct reduction to take place in zones of higher temperature. By the time the materials reach the lower section of the stack they have been reduced to iron sponge and are entering the melting zone completely surrounded by a CO gas phase in the presence of excess carbon. Under these conditions the melting iron is not exposed to any oxidizing influences. Because the combustion zone is separate and independent of 135 the melting column, its temperature can be regulated and can be maintained uniformly at a point most advantageous to the production of high grade metal. This is not the case in the blast furnace where the materials descend directly into the combustion zone in a more or less irregular manner.

While I preferably use a combustion chamber 140 of annular shape, other forms, such as elliptical or rectangular, can be employed for the same 145 150

purpose. In case of iron ores being used, I may charge them in their natural state or dried or sintered or briquetted, or I may mix crushed lump ores with fines and briquettes. With varying 5 character of ores, various methods will be found desirable. In any case, my invention provides a means of producing iron or steel from ores, scrap or sponge iron which neither become re-oxidized with the blast nor saturated with carbon as happens in the present blast furnaces. The saturation of iron with carbon in the blast furnace necessitates a subsequent oxidation process in the Bessemer converter or open hearth furnace, which again exposes the metal to vitiation with oxides. By my method the amount of 10 carbon which the metal absorbs can be kept under control and can be limited to small amounts and the carbon can be reduced by the addition of iron ore, either in the hearth or preferably 15 at the top, as lumps of sufficient size that they will arrive in the molten bath containing the iron oxide required to bring down the carbon in the metal to the desired point. It is a well known 20 fact that the removal of carbon by iron oxide 25 added to the bath results in a finer grade of steel than if the carbon is removed by an air blast, as in the Bessemer process.

The form of construction shown in the drawings is to be understood to be illustrative only, 30 as my improved method may be carried out in furnaces differing materially from that shown, and I contemplate such changes and modifica-

tions, both in the process and in the apparatus for carrying out, as may come within the spirit and scope of the appended claims.

I claim:

1. The method of metal production, which comprises treating a column of descending ore by surrounding the lower portion of the column with a reducing flame adjacent and spaced from the column of material, the reducing flame being created by the injection of fuel and air, the flame being maintained at a temperature sufficient to melt the reduced ore in the lower portion of the column of material, supporting the column of material out of contact with the melted metal, and passing reduced gases from the flame up through the upper portion of the column whereby the ore in the column is reduced. 80
2. The method of producing pure metal, which comprises treating a column of descending ore by surrounding the lower portion of the column with a reducing flame adjacent and spaced from the column of material, the reducing flame being created by the injection of fuel and air, the flame being maintained at a temperature sufficient to melt the reduced ore in the lower portion of the column of material, supporting the column of material out of contact with the melted metal, treating the molten metal with a refining flame, and passing reducing gases from the flame up through the upper portion of the column whereby the ore in the column is reduced. 85 90 95 100 105

HERMAN A. BRASSERT.

35

40

45

50

55

60

65

70

75

110

115

120

125

130

135

140

145

150